

Aug. 17, 1954

E. B. STORY

2,686,742

METHOD OF MAKING A WROUGHT IRON PRODUCT

Filed April 20, 1953



Fig. 1.



Fig. 2.



Fig. 3.



Fig. 4



Fig. 5

INVENTOR

EDWARD B. STORY

*By Hayes, Leonard & Burrell  
his attorneys*

## UNITED STATES PATENT OFFICE

2,686,742

## METHOD OF MAKING A WROUGHT IRON PRODUCT

Edward B. Story, Bethel, Pa., assignor to A. M. Byers Company, Pittsburgh, Pa., a corporation of Pennsylvania

Application April 20, 1953, Serial No. 349,806

4 Claims. (Cl. 148—12)

1

This invention relates to a method of making a wrought iron product involving fragmenting elongated slag fibers of wrought iron by working the wrought iron at a temperature below the temperature at which the slag fibers are substantially deformable without fragmenting, or, in other words, below the temperature at which the slag fibers lose their plasticity, and coalescing the fragmented slag fibers. This application is in part a continuation of my copending application Serial No. 155,975, filed April 14, 1950, now abandoned, which is in turn in part a continuation of my application Serial No. 7,837, filed February 12, 1948, now abandoned, which was copending therewith.

In the manufacture of wrought iron the practice has been to hot roll the wrought iron to elongate the slag inclusions to produce relatively fine elongated slag fibers. The wrought iron thus produced has been characterized by high longitudinal ductility and low transverse ductility. I have discovered how to make a wrought iron product with longitudinal ductility as high as before and with transverse ductility very much higher than has previously been obtained. I make a wrought iron product out of wrought iron having elongated slag fibers by fragmenting the elongated slag fibers by working the wrought iron at a temperature below 1900° F. and thereafter coalescing the fragmented slag fibers by annealing the wrought iron at a temperature at least about 1900° F. The result of the fragmenting and coalescing of the slag fibers is to produce in the wrought iron a transverse ductility which may be of the order of a multiple of the best transverse ductility previously thought possible. While I prefer to work the wrought iron at a temperature below 1900° F. by rolling it in the longitudinal direction, the working to fragment the elongated slag fibers can be accomplished otherwise, as, for example, by drawing.

In a preferred method of making a rolled wrought iron product I roll wrought iron generally parallel to an axis in the wrought iron and while the wrought iron is at a temperature below 1900° F., continue said rolling until slag fibers of the wrought iron fragment and thereafter coalesce the fragmented slag fibers by annealing the wrought iron at a temperature at least about 1900° F. I preferably continue said rolling until the thickness of the wrought iron has been reduced at least about 10%, and in a further preferred method I continue said rolling until the thickness of the wrought iron is not substantially greater than one-half of the thickness of the

2

wrought iron at the beginning of said rolling. I find that the extent of working to accomplish fragmenting of the elongated slag fibers varies with the temperature at which the working is effected. For example, when the working is effected at a temperature only slightly below 1900° F. a more drastic working is required to fragment the slag fibers than when the working temperature is lower. I find that when the working to fragment the slag fibers is effected at a temperature of the order of 1600° F. the reduction to accomplish the desired result should be at least about 50%. When the working is effected at room temperature a reduction of 10% or less may be sufficient.

The accompanying drawings are photomicrographs of conventional wrought iron and wrought iron made in accordance with my improved method above described and specifically by rolling.

In the drawings

Figure 1 is a photomicrograph at one hundred magnifications of a section of conventionally rolled wrought iron, the section being taken parallel to the direction of rolling;

Figure 2 is a photomicrograph at one thousand magnifications of a section of conventionally rolled wrought iron, the section being taken parallel to the direction of rolling;

Figure 3 is a photomicrograph at one hundred magnifications of a section of wrought iron made in accordance with the improved method above described, the wrought iron having been annealed at a temperature above the temperature at which the slag inclusions lose their plasticity, the section being taken parallel to the direction of rolling;

Figure 4 is a photomicrograph at one thousand magnifications of a section of wrought iron made in accordance with the improved method above described except that the wrought iron shown was not annealed at a temperature above the temperature at which the slag inclusions lose their plasticity, the section being taken parallel to the direction of rolling; and

Figure 5 is a photomicrograph at one thousand magnifications of a section of wrought iron made in accordance with the improved method above described, the wrought iron having been annealed at a temperature above the temperature at which the slag inclusions lose their plasticity, the section being taken parallel to the direction of rolling; in other words, Figure 5 illustrates the result of coalescing the fractured slag fibers of the wrought iron of Figure 4 by annealing at a temperature at least about 1900° F.

Figure 1 is, as above stated, a photomicrograph at one hundred magnifications of a section of conventionally rolled wrought iron, the section being taken parallel to the direction of rolling. It is a representative section for heavily conventionally rolled wrought iron, to wit, wrought iron which is unidirectionally rolled almost entirely at temperatures above the temperature at which the slag inclusions lose their plasticity. That temperature is in the vicinity of 1900° F. The slag fibers in Figure 1 are designated by reference numeral 2. They are relatively long stringy masses of slag whose shape comes about through hot rolling of the wrought iron. The slag masses of Figure 1 are not fragmented or fractured; in some cases they are "necked off" by the hot rolling, i. e., by being rolled so thin that they separate while still plastic into individual aligned long stringy fibers.

To show more clearly the character of the slag fibers in conventionally rolled wrought iron I have provided Figure 2 which, as above stated, is a photomicrograph at one thousand magnifications of a section of conventionally rolled wrought iron, the section being taken parallel to the direction of rolling. The slag fibers are indicated by reference numeral 2 in Figure 2. They are long stringy slag masses oriented generally parallel to the direction of rolling. The long stringy slag fibers considerably reduce the transverse tensile strength and ductility of the wrought iron. Conventionally unidirectionally rolled wrought iron shows a ductility or elongation of about 5% or less in a transverse tension test. The best transverse ductility of conventionally unidirectionally rolled wrought iron is less than 7%.

Figure 3 is a photomicrograph at one hundred magnifications of a section of wrought iron made in accordance with my improved method, the wrought iron having been annealed at a temperature above the temperature at which the slag inclusions lose their plasticity, the section being taken parallel to the direction of rolling. The reduction of the wrought iron shown in Figure 3 has been effected largely at temperatures below the temperature at which the slag fibers lose their plasticity, to wit, largely below 1900° F. The rolling fractures or fragments the elongated slag fibers into a series of slag masses which are aligned in the direction of rolling. A single long stringy slag fiber existing at 1900° F. may fracture into a large number of aligned masses as the rolling continues below 1900° F.

Figure 4 is a photomicrograph at one thousand magnifications of a section of wrought iron made in accordance with my improved method above described except that the wrought iron shown was not annealed at a temperature above the temperature at which the slag inclusions lose their plasticity, the section being taken parallel to the direction of rolling. The fractured slag masses are clearly shown in Figure 4 but they assume a shape which is more rectangular or block-like in cross section than spherical. They are designated by reference numeral 4.

Figure 5 is a photomicrograph at one thousand magnifications of a section of wrought iron as shown in Figure 3 clearly illustrating the separate aligned slag masses formed by fracturing non-plastic long stringy slag fibers. The wrought iron shown in Figures 3 and 5 has been heat treated at a temperature above the temperature at which the slag inclusions lose their plasticity, i. e., at a temperature above 1900° F., for ex-

ample, 2000° F. The heat treatment coalesces or nodulizes the slag masses formed by fracturing of the original long stringy slag fibers. Those masses assume generally round or spherical shape as shown in both Figure 3 and Figure 5 but more clearly in the latter figure. The slag nodules are designated by reference numeral 3 in Figures 3 and 5. Figure 5 shows the result of heat treating at a temperature above 1900° F. of wrought iron as shown in Figure 4. The generally rectangular or block-like slag masses coalesce or nodulize into masses which are more nearly spherical in shape. The coalescing or nodulizing of the slag fibers is accompanied by some increase in the spaces therebetween with a consequent increase in transverse ductility of the wrought iron.

The transverse ductility of wrought iron made by my improved process is much higher than the transverse ductility of conventionally unidirectionally rolled wrought iron and may be several times as great. A typical specimen of wrought iron as shown in Figure 3 displays a transverse elongation of about 17% or in the neighborhood of three times the transverse elongation of very good conventionally unidirectionally rolled wrought iron. My improved wrought iron shows a transverse elongation of a minimum of about 7% which is better than the best transverse elongation of conventionally unidirectionally rolled wrought iron. The ductilities are measured by the percentage elongation in a standard tension test in a gauge length of 8" of a transverse test specimen of normal cross section. The cross-sectional dimensions of the test specimen may, for example, be of the order of 1.5" x .1".

While I greatly improve the transverse properties of wrought iron the longitudinal properties remain approximately the same as the longitudinal properties of conventionally unidirectionally rolled wrought iron. Thus my wrought iron suffers nothing in longitudinal properties while being improved as much as threefold in transverse properties.

In a preferred method of procedure I may heat a wrought iron billet to about 2500° F. and roll the billet until the temperature of the wrought iron has fallen to a temperature substantially lower than 1900° F. After the wrought iron cools below 1900° F. the slag inclusions lose their plasticity and upon further rolling they are fractured or torn apart as above described into masses each having a dimension in the direction of alignment equal to a minor fraction of the length of the original fiber. The slag masses are aligned in the direction of rolling and in the direction of the length of the original fibers. They are of generally block-like appearance in a cross section taken parallel to the direction of rolling as shown in Figure 4. As indicated above, if the rolling is effected at temperatures only slightly lower than 1900° F. the rolling is desirably continued until the thickness of the wrought iron is not substantially greater than one-half of the thickness of the wrought iron at the beginning of the portion of the rolling following cooling of the wrought iron to 1900° F. which insures fragmentation of a substantial number of slag fibers. As already explained, the extent of rolling or other working to accomplish the desired fragmentation of the slag fibers may be substantially reduced as the temperature is reduced. The thus rolled wrought iron is annealed by heating it to 1900° F. or some-

what higher to cause the slag fragments to coalesce with the advantages above explained.

By my invention I can produce by unidirectional rolling without reheating wrought iron whose transverse ductility is far greater than the transverse ductility of conventionally unidirectionally rolled wrought iron and at least as high as the ductility in either crosswise direction of cross rolled wrought iron whose ductility in both directions of rolling at right angles to each other is about the same. The longitudinal ductility of my improved wrought iron is very much greater than the ductility in the respective directions of rolling of cross rolled wrought iron and is at least equal to the longitudinal ductility of most conventionally unidirectionally rolled wrought iron. The rolled product may be of any desired length, no limit being imposed on its length except by the size of billet which can be produced and rolled.

The improved product of my invention has many uses and is of wide utility. As an example, it is ideally suited for heat exchanger pipe which is thin walled tubing whose ends pass through holes in tube sheets and are rolled back against the sheets. When my improved method is employed in making the wrought iron heat exchanger tubing of any desired length may be produced and may be rolled over against the tube sheet without danger of splitting.

While I have shown and described a present preferred method of practicing my invention it is to be distinctly understood that the invention is not limited thereto but may be otherwise variously practiced within the scope of the following claims.

I claim:

1. A method of making a wrought iron product out of wrought iron having elongated slag fibers comprising fragmenting the elongated slag fibers by working the wrought iron at a temperature

below 1900° F. and thereafter coalescing the fragmented slag fibers by annealing the wrought iron at a temperature at least about 1900° F.

- 5 2. A method of making a rolled wrought iron product comprising rolling wrought iron generally parallel to an axis in the wrought iron and while the wrought iron is at a temperature below 1900° F., continuing said rolling until slag fibers of the wrought iron fragment and thereafter coalescing the fragmented slag fibers by annealing 10 the wrought iron at a temperature at least about 1900° F.
- 15 3. A method of making a rolled wrought iron product comprising rolling wrought iron generally parallel to an axis in the wrought iron and while the wrought iron is at room temperature, continuing said rolling until the thickness of the wrought iron has been reduced about 10% and annealing the wrought iron at a temperature at least about 1900° F.
- 20 4. A method of making a rolled wrought iron product comprising rolling wrought iron generally parallel to an axis in the wrought iron and while the wrought iron is at a temperature below 1900° F., continuing said rolling until the thickness 25 of the wrought iron is not substantially greater than one-half of the thickness of the wrought iron at the beginning of said rolling and annealing the wrought iron at a temperature at least about 1900° F.

30 References Cited in the file of this patent

UNITED STATES PATENTS

| Number    | Name    | Date          |
|-----------|---------|---------------|
| Re. 7,003 | Lauth   | Mar. 21, 1876 |
| 35 826    | Johnson | July 9, 1838  |
| 2,335,506 | Grange  | Nov. 30, 1946 |

OTHER REFERENCES

40 "The Making, Shaping and Treating of Steel," publ. by U. S. Steel Corp., 1940, pages 310, 311, 327.